

R. L. WHITEHEAD,  
CASTING ELECTRODES,  
APPLICATION FILED JUNE 26, 1914.

1,206,964.

Patented Dec. 5, 1916.



Fig. 2,



WITNESSES

*W. H. BREWER*  
K. M. Schuy  
L. B. Schuyler

**INVENTOR:**

INVENTOR,  
Robert L. Whitehead,  
BY  
Kenne, Davis & Goldfarb,  
ATTORNEYS

R. L. WHITEHEAD,  
CASTING ELECTRODES,  
APPLICATION FILED JUNE 26, 1914.

1,206,964.

Patented Dec. 5, 1916.  
2 SHEETS—SHEET 2.

Fig. 3,



Fig. 4,



Fig. 5,



Fig. 6,



WITNESSES

K. M. Schulz  
J. B. Schroeder

Fig. 7,



INVENTOR:

Robert L. Whitehead,  
BY

Janine, Davis & Goldsberry,  
ATTORNEYS

## UNITED STATES PATENT OFFICE.

ROBERT L. WHITEHEAD, OF PERTH AMBOY, NEW JERSEY, ASSIGNOR TO AMERICAN SMELTING & REFINING COMPANY, OF MAURER, NEW JERSEY, A CORPORATION OF NEW JERSEY.

## CASTING ELECTRODES.

1,206,964.

Specification of Letters Patent.

Patented Dec. 5, 1916.

Application filed June 26, 1914. Serial No. 847,372.

*To all whom it may concern:*

Be it known that I, ROBERT L. WHITEHEAD, a citizen of the United States, residing at Perth Amboy, county of Middlesex, 5 State of New Jersey, have invented certain new and useful Improvements in Casting Electrodes; and I do hereby declare the following to be a full, clear, and exact description of the invention, such as will enable others skilled in the art to which it appertains to make and use the same.

My invention relates to certain new and useful improvements in the casting of electrodes and is particularly applicable to the 15 casting of anodes to be used in the electrolytic production of pure metal, as, for instance, in the production of electrolytically deposited copper.

In electrolytic processes for the recovery 20 of copper and like metals, it is customary to cast the crude metal in shallow open top molds, carried upon a rotating support and which are filled in succession from a stationary source of supply of the melted metal. 25 The anodes thus produced have integral lugs which serve as supports for suspending them in the electrolytic vats and which rest upon the bus bars which supply the working current to the apparatus and which also rest 30 upon intermediate insulating strips parallel to the bus bars along the upper ends of the dividing partitions between the series of depositing vats.

In order to provide a highly efficient and 35 reliable electrical connection between the supply bus bar and the individual anodes, or between each individual anode and its connecting cathode across the series of depositing vats, I provide a ridge or projection, 40 on one of the anode lugs, which ridge or projection coöperates with a recess in the coöperating lug of the cathode, the arrangement being such that the walls of the recess will come in wedging contact at their lower 45 edges with the projection or ridge on the anode lug, suitable clearance being provided beyond the contacting surfaces; all as set forth more fully in my application for Letters Patent of the United States, Serial 50 Number 747,253, filed February 10, 1913, for improvements in electrolytic apparatus.

The present invention is designed to provide a casting mold for producing anodes whose contact-making lugs are provided 55 with the ridge or projection referred to.

In the accompanying drawings,—Figure 1 represents a top plan view of an open top mold constructed in accordance with my invention; Fig. 2 represents a fragmentary view thereof, likewise in plan, and on a larger scale; Fig. 3 represents a sectional view on the dotted line 3—3 of Fig. 1; Figs. 4 and 5 represent respectively, sectional views, on an enlarged scale, on the dotted lines 4—4 and 5—5 respectively, of Fig. 2; Fig. 6 represents a top plan view of a portion of the anode lug with its ridge or projection, as produced in the casting mold; Fig. 7 represents a section thereof, on the line 7—7, of Fig. 6; and Fig. 8 represents a side elevation of the end of the lug, with its contact ridge or projection.

Similar letters of reference indicate similar parts throughout the several views.

Referring to the drawings, *a* represents the main body portion of the open shallow mold, which is provided with suitable strengthening ribs *a'*, as shown. The mold is provided further with the wings or extensions *b*, *c*, for casting the supporting lugs, *b* being shown as adapted for the casting of the contact ridge or projection upon the corresponding anode lug.

It will be noted that the outer walls of the main body portion of the mold have an upward and outward incline, and that this incline likewise extends into the wings *b*, *c*. The purpose of this incline is to afford a sufficient draft to permit the ready removal of the cast anode from the mold at the completion of the casting operation. The corresponding surfaces of the anode will have a like inclination, as will be evident. This is not desirable, however, for the contact ridge or projection *e* of the lug *f*, which lug is the one to be cast in the wing *c* of the mold. On the contrary, it is preferable that the ridge or projection *e* should be substantially vertical along its top edge *g*, as drawn from the mold, in order that said edge *g* and also the inclined faces of the ridge or projection should not suffer distortion in cooling. In order to compensate for any such tendency to distortion, I so fashion the walls of the mold that on both sides of the recess *h* in which the projection *e* is to be cast there is provided a tapering vertical recess *i*. In consequence of the provision of these supplemental recesses *i* the contact

# BEST AVAILABLE COPY

1,208,984

ridge or projection *e* is flanked at its base and along opposite sides thereof with a basal fillet *n*. The function of these fillets is to provide, at the base of the contact ridge or projection and on both sides thereof, a body of metal sufficient to prevent the more or less unequal shrinking which is liable to occur in the contact ridge or projection in those instances where the fillets referred to 10 are not present and where the ridge or projection springs directly from the inclined side *m* of the supporting lug. The presence of the fillets *n* supplies a body of metal of gradually increasing thickness, corresponding 15 to the inclination of the side *m* of the supporting lug, and obviates unequal shrinkage in the ridge or projection, for the reason that as the cross-sectional area of the lug *f* decreases, the cross-sectional area of the 20 fillets increases. This compensating action of the fillets does not, however, interfere with the drawing of the lug *f* from the mold, inasmuch as although the shrinkage in the ridge or projection *e* is rendered sub- 25 stantially uniform by the presence of the fillets *n*, such shrinkage, because of the limited size of the fillets is nevertheless sufficient to permit the cast ridge or projection, on cooling, to withdraw itself from contact 30 with the walls of the recess *h* to the necessary degree to clear the mold and permit the stripping of the casting therefrom.

What I claim is:

1. A mold for casting a contact ridge or projection upon the supporting lug of an electrode, said mold being provided with a lug-casting wing having inclined sides for its casting cavity thereby facilitating the drawing of the lug, and being further provided with a recess having vertical walls and within which the contact ridge or projection is to be cast and with supplemental fillet-forming recesses at opposite sides of the contact ridge recess, whereby on cooling 45 of the casting with resultant shrinkage, the presence of the fillets formed by the fillet-forming recesses will cause the walls of the contact ridge or projection to remain vertical.
- 50 2. A mold for casting a contact ridge or projection upon the supporting lug of an electrode, said mold being provided with a lug-casting wing having inclined sides for its casting cavity thereby facilitating the

drawing of the lug, and being further provided with a recess having vertical walls and within which the contact ridge or projection is to be cast and with supplemental fillet-forming recesses at opposite sides of the contact ridge recess, said supplemental 60 fillet-forming recesses increasing in area in cross-section from above downwardly, whereby on cooling of the casting with resultant shrinkage, the presence of the fillets formed by the fillet-forming recesses will cause the walls of the contact ridge or projection to remain vertical.

3. The method of casting a substantially flat article, such as a copper anode for use in electrolytic refining, having its edges inclined relatively to the general plane of the casting to facilitate removal of the casting from the mold and having a contact ridge or projection thereon, the walls of which are transverse to the general plane of the casting, including the casting of fillets at opposite sides of the base of the said contact ridge or projection, whereby on cooling of the casting with resultant shrinkage, the presence of the metal of the said fillets 70 will maintain the walls of the contact ridge or projection transverse to the general plane of the casting.

4. The method of casting a substantially flat article, such as a copper anode for use in electrolytic refining, having its edges inclined relatively to the general plane of the casting to facilitate removal of the casting from the mold and having a contact ridge or projection thereon, the walls of which are 75 transverse to the general plane of the casting, including the casting of fillets at opposite sides of the base of the said contact ridge or projection, which fillets are increased in cross-section throughout their 80 length in correspondence with the inclination of the edges of the casting, whereby on cooling of the casting with resultant shrinkage, the presence of the metal of the said fillets will maintain the walls of the contact 85 ridge or projection transverse to the general plane of the casting.

In testimony whereof I affix my signature, in presence of two witnesses.

ROBERT L. WHITEHEAD,

Witnesses:

M. A. BILL,

VIOLET C. BENNETT.